

(No Model.)

L. G. CLAUDE.

HORSESHOE.

No. 329,141.

Patented Oct. 27, 1885.

Fig. 1.



Fig. 3.



Fig. 2.



Fig. 4.



Fig. 5.



Fig. 6.



WITNESSES:

*E. B. Bolton  
Bookbinder*

INVENTOR:

*Louis G. Claude,  
By his Attorneys,  
Burke, Fraser & Sonnleitner*

# UNITED STATES PATENT OFFICE.

LOUIS G. CLAUDE, OF NEW YORK, N. Y., ASSIGNOR, BY MESNE ASSIGNMENTS,  
TO THE RUSSELL HORSESHOE COMPANY, OF SAME PLACE.

## HORSESHOE.

SPECIFICATION forming part of Letters Patent No. 329,141, dated October 27, 1885.

Application filed December 23, 1884. Serial No. 151,042. (No model.)

*To all whom it may concern:*

Be it known that I, LOUIS G. CLAUDE, a citizen of the United States, residing in the city, county, and State of New York, have invented certain new and useful Improvements 5 in Horseshoes, of which the following is a specification.

This invention relates to machine-made horseshoes, and has special reference to those 10 made of combined iron and steel with solid calks.

Figure 1 of the accompanying drawings is a plan of the upper side of my improved horseshoe in its preferred form. Fig. 2 is a side 15 elevation thereof. Fig. 3 is a plan of the under side of the shoe, and Fig. 4 is a front elevation of the same. Fig. 5 is a plan of the under side of a modified construction of shoe, and Fig. 6 is a side elevation thereof.

20 In all the figures the white portions of the shoes designate steel, and the dark portions, shaded with a tint of ruled lines, designate iron.

I will first describe in detail the shoe shown 25 in Figs. 1 to 4. The body of the shoe is a flat plate, A, of the curved outline shown, and integral with it are the toe-calks B and heel-calks C C. The grain or fiber of the metal extends in a straight or parallel direction longitudinally of the shoe, and consequently crossing 30 its toe portion in a direction substantially transverse to the outline thereof. At this portion, which is the only part of the shoe where the grain of the metal crosses it transversely, the shoe is thickened by the toe-calk B, which extends across the toe transversely to the grain of the metal, and is preferably elongated laterally of the shoe, as shown. Through the middle of the toe and toe-calk 35 passes a stripe or streak, a, of iron, and on each side of this and parallel with it are two streaks or cores, b b, of steel, which extend from the front edge of the shoe across the toe portion and down each leg, on the inner side thereof, to the heel. Outside of these steel portions 40 are flanks c c of iron, which extend along the outer sides of the shoe to the heels. The toe-calk B extends across the iron center a, and its ends are formed of the steel portions b b. 45 The heel-calks C C are formed mainly of the steel portions b b, and the outer side of each

is formed of the iron portions c c. At the extreme toe of the shoe the usual toe-clip, D, extends upwardly, being formed wholly from the iron center a. The upper side of the plate A 55 is formed with the usual "concave" or bevel, d, and in the underside of the plate are formed the usual "creases," e e, close along each outer margin, for the nail-heads. Through the bottom of these creases the usual nail-holes, f f, are 60 punched.

This improved shoe possesses the following characteristic advantages: The grain of the metal extending longitudinally of the shoe renders the sides or legs where they are not 65 strengthened by the projecting calks as strong as possible for their weight, and the grain, by extending in parallel and substantially straight direction, is under no strain, as in those shoes where the fiber of the metal is distorted or 70 disturbed by bending or other violent manipulation. For the same reason the respective iron and steel portions are not liable to separate, as in a bent shoe, thus avoiding the slivering of the outer layers or portions. The toe-calk, by being made to extend across the greater 75 portion of the toe of the shoe, strengthens the only part that might otherwise be weak by reason of the grain of the metal extending transversely to it. The outer flanks of iron afford 80 a soft and malleable substance in which to form the creases and punch the nail-holes, it being impracticable to punch these through the steel portion of the shoe. The iron center affords a ductile substance from which to 85 strike up or swage the toe-clip, and the clip formed thus of iron is less brittle than if of steel, and the iron center also, by extending through the toe-calk, renders the middle portion thereof softer than the ends, which are of 90 steel, and consequently the iron middle wears away faster in use than the steel ends, leaving the latter standing, and retaining thus a firm foothold for the horse. Fig. 4 show this result graphically, the dotted line x x denoting 95 the outline of the toe-calk after having been subjected to a certain amount of wear.

This shoe is made as follows: An ingot is first built up of two steel cores separated by and enveloped by bars or plates of wrought-iron. This is heated and rolled down until a flat plate or bar is made of a width 100

somewhat greater than that of the finished shoe and as thick as the shoe is through its calks. This bar is then passed while hot between special rolls, which reduce it at once 5 to the thickness of the plate A between the calks, leaving the calks standing. These operations are fully described in my application executed this day for patent on "im- 10 provements in bars of combined iron and steel and their manufacture," application No. 150,778, filed December 19, 1884. The same operation also forms the concaves in the upper side of the bar. The shoes are next 15 punched out of this bar, following one another heel to toe, the shoe-blanks thus formed hav- 20 ing each the same outline as the finished shoe, except that their heels are wider apart, and their toe has a slight projection to form the toe-clip. The heels of each shoe are then squeezed 25 together against a former. The creases are then formed and the toe-clip is then struck up by a swaging-roller. All these operations are described in my application for patent ex- 30 ecuted this day entitled "improvements in the manufacture of horseshoes with solid calks," application No. 150,889, filed December 20, 1884, and the three operations last named are best performed by the machine disclosed in 35 my application for patent on "improvements in horseshoe-machines," application No. 151,134, filed December 26, 1884. Finally, the nail-holes are punched, preferably one at 40 a time, by a punching-press.

The modified shoe shown in Figs. 5 and 6 is 45 what is known as a "flat" shoe, being nearly devoid of calks, or, more correctly, being formed with extremely low calks. The calks B and C C are beveled off gradually on their rear sides and have an abrupt front side, 50 thereby rendering the toe of the shoe enough thicker than the remaining portions to prevent its wearing off before the shoe is otherwise worn out. The toe will be prevented from wearing away faster at the sides than 55 in the middle, and thereby acquiring a rocker form by the iron center, the steel sides remaining sharp after the center has worn down below them. In this shoe the grain of the metal extends quite straight through the 60 heel portion, as shown, instead of curving inwardly. This is due to the shoe being stamped out originally of the exact outline desired, thereby avoiding the pressing of the heels together; but the former method is preferable. 65

55 My invention may be in part availed of in making a shoe of all iron or all steel; but the shoe made of the combined metals, as described, is preferable.

What I claim, and desire to secured by Let- 60 ters Patent, is—

1. A horseshoe of wrought metal, wherein the grain of the metal extends in parallel and substantially straight direction longitudinally of the shoe, substantially as specified.

2. A horseshoe of wrought metal, wherein the grain of the metal extends in parallel direction, crossing the toe portion thereof longitudinally of the shoe, and extending through the heel portions thereof with a slight inward deflection substantially parallel with the outlines 70 of the heel portions, as specified.

3. A horseshoe of wrought metal, wherein the grain of the metal extends in parallel direction longitudinally of the shoe, and crossing the toe portion thereof transversely to its out- 75 line, and provided with a toe-calk extending across its toe portion transversely to the grain of the metal, thereby strengthening the toe- portion, substantially as set forth.

4. A horseshoe of alternate strips of iron 80 and steel, wherein the grain of the metal ex- tends in substantially parallel direction longitu- dinally of the shoe, and calk projections are formed in the steel portions of the shoe, sub- stantially as set forth.

5. A horseshoe of combined iron and steel, 85 wherein the grain of the metal extends in par- allel direction longitudinally of the shoe, the middle of the toe portion of the shoe being of iron, and the toe-clip being formed from such 90 iron middle, substantially as set forth.

6. A horseshoe of wrought metal having a 95 toe-calk of combined iron and steel, the ends of the calk being of steel and its middle of iron, whereby the middle wears away faster in use than the ends, substantially as set forth.

7. A horseshoe of combined iron and steel, 100 wherein the grain of the metal extends in par- allel direction longitudinally of the shoe, cross- ing the toe portion transversely to the outline thereof, having steel sides and iron flanks, whereby the creases and nail-holes are formed in the iron flanks, substantially as set forth.

8. A horseshoe of combined iron and steel, 105 wherein the grain of the metal extends in par- allel direction longitudinally of the shoe, and consisting of a middle stripe, a, of iron, side stripes or cores, b b, of steel, and flanks c c of iron, substantially as set forth.

In witness whereof I have hereunto signed 110 my name in the presence of two subscribing witnesses.

LOUIS G. CLAUDE.

Witnesses:

ARTHUR C. FRASER,  
HENRY CONNETT.